

# United States Patent [19]

Cho

[11] Patent Number: 4,927,470

[45] Date of Patent: May 22, 1990

[54] THIN GAUGE ALUMINUM PLATE  
PRODUCT BY ISOTHERMAL TREATMENT  
AND RAMP ANNEAL

[75] Inventor: Alex Cho, Richmond, Va.

[73] Assignee: Aluminum Company of America,  
Pittsburgh, Pa.

[21] Appl. No.: 256,840

[22] Filed: Oct. 12, 1988

[51] Int. Cl.<sup>5</sup> ..... C22F 1/04

[52] U.S. Cl. ..... 148/12.7 A; 148/415;  
148/417; 148/439; 148/440

[58] Field of Search ..... 148/12.7 A, 2, 415,  
148/417, 439, 440

## [56] References Cited

### U.S. PATENT DOCUMENTS

4,092,181 5/1978 Paton et al. ..... 148/12.7 A

Primary Examiner—R. Dean

Attorney, Agent, or Firm—Andrew Alexander

## [57] ABSTRACT

Disclosed is a method of producing an unrecrystallized aluminum base, wrought product having improved levels of strength and fracture toughness. The method comprises providing a body of the aluminum base alloy, hot working the body to a wrought product and then subjecting it to an isothermal soak followed by a ramp anneal.

60 Claims, 1 Drawing Sheet





THIN GAUGE ALUMINUM PLATE PRODUCT BY  
ISOTHERMAL TREATMENT AND RAMP  
ANNEAL

INTRODUCTION

This invention relates to heat treatable alloys such as the 2000, 6000 and 7000 series alloys and more specifically, it relates to thermal mechanical processing of such alloys to improve strength and fracture toughness in thin plate, for example.

For many years, alloys of the 7000 series have been used for high strength and toughness in aerospace applications. These alloys can be age hardened to very high strengths, for example, in the T6 temper condition. Further, the strengths of these alloys may be increased by increasing solute content. Increasing the strength of these alloys permits designers to reduce the weight of aircraft by reducing thickness of load carrying components such as upper wing skins. Such components must have (and even demand) relatively high fracture toughness as well as high strength to be useful. Several sources indicate that plate having an unrecrystallized structure develops higher toughness than plate having a recrystallized structure. It is well known by those skilled in the art that maintaining the rolling temperature at a high level, typically above about 750° F., allows the aluminum alloy to dynamically recover with a fine subgrain structure, typically about 1 to 2  $\mu$ m. This dynamically recovered structure is resistant to recrystallization during subsequent solution heat treatment. However, as the increased strength and toughness allows the use of thinner gauges, prior fabricating techniques and thermal mechanical practices often do not permit production of such products with an unrecrystallized structure because of the tendency for the rolling temperature to fall as the plate thickness is reduced.

Prior art teaches how to achieve recrystallized grain structure but not how to achieve unrecrystallized structure. In the prior art, U.S. Pat. No. 4,092,181 discloses a method of imparting a fine grain recrystallized structure to aluminum alloys having precipitating constituents. The method is provided for imparting a fine grain structure to aluminum alloys which have precipitating constituents. The alloy is first heated to a solid solution temperature to dissolve the precipitating constituents in the alloy. The alloy is then cooled, preferably by water quenching, to below the solution temperature and then overaged to form precipitates by heating it above the precipitation hardening temperature for the alloy but below its solution treating temperature. Strain energy is introduced into the alloy by plastically deforming it at or below the overaging temperature used. The alloy is then subsequently held at a recrystallization temperature so that the new grains are nucleated by the overaged precipitates and the development of these grains results in a fine recrystallized grain structure. This structure is useful for imparting superplastic properties but will provide lower toughness than an unrecrystallized structure.

In contrast, the present invention provides improved thermal mechanical processing techniques which permit the fabrication of flat rolled products, particularly thin gauge plate and sheet 7000 series aluminum alloys having a substantially unrecrystallized structure which imparts to the plate improved combinations of strength and fracture toughness.

SUMMARY OF THE INVENTION

A principal object of this invention is to provide an improved aluminum based, heat treatable, flat rolled product.

Another object of this invention is to provide an unrecrystallized, 7000 series alloy, thin gauge plate or sheet product.

Yet another object of this invention is to provide a process for making an unrecrystallized, 7000 series alloy, thin gauge flat rolled product.

These and other objects will become apparent from the specification, drawings and claims appended hereto.

In accordance with these objects, there is provided an unrecrystallized thin gauge flat rolled product suitable for fabricating into aircraft structural members, the unrecrystallized thin gauge flat rolled product comprised of aluminum base alloy consisting essentially of 1.0 to 12 wt. % Zn, 0.5 to 4.0 wt. % Mg, max. 3.0 wt. % Cu, max. 1.0 wt. % Mn, max. 0.5 wt. % each of Si, Fe, Cr, Ti, Zr, Sc and Hf, the balance aluminum and impurities.

Also, there is provided a method of producing an unrecrystallized aluminum base alloy, thin gauge flat rolled product which includes hot working a body of the alloy to a final gauge flat rolled product. This is followed by isothermal soaking the product, ramp annealing, solution heat treating, quenching and aging to provide a substantially unrecrystallized product having improved levels of strength and fracture toughness.

BRIEF DESCRIPTION OF THE DRAWING

The sole FIGURE is a schematic representing steps in the process for producing thin gauge unrecrystallized plate in accordance with the invention.

DETAILED DESCRIPTION OF THE PREFERRED EMBODIMENTS

Aluminum based alloys which respond to thermal mechanical processing in accordance with the present invention include the Aluminum Association 7000 series. Such alloys include, for example, 7050, 7150, 7075, 7475, 7049 and 7039.

Typically, these aluminum based alloys contain 1.0 to 12.0 wt. % Zn, 0.5 to 4.0 wt. % Mg, max. 3.0 wt. % Cu, max. 1.0 wt. % Mn, max. 0.5 wt. % each of Si, Fe, Cr, Ti, Zr, Sc, and Hf, the balance aluminum, incidental elements and impurities. These alloys may be referred to as Al—Zn—Mg or Al—Zn—Cu—Mg type. Alloys which seem to respond more readily to thermal mechanical processing in accordance with the present invention include higher levels of zinc, preferably 7.0 to 12.0 wt. % Zn with a typical level being 8.0 to 11.0 wt. %. Magnesium at these levels of zinc can range from 0.2 to 3.5, preferably 0.4 to 3.0 wt. %. Also, copper at the higher zinc levels can range from 0.5 to 3.0 wt. %, preferably 1.0 to 3.0 wt. %. These alloying elements may be higher in certain cases, but the resulting alloys can have low fracture toughness. In certain cases, other ranges of alloying elements may be preferred. For example, Zn can be in the range of 7.0 to 9.0 wt. %, Mg 1.5 to 2.5 wt. %, Cu 1.9 to 2.7 wt. %, Zr, 0.08 to 0.14, with impurities such as Fe and Si being less than 0.3 wt. %.

While the AA7000 series aluminum alloys have been described in detail, it will be understood that the invention can be applied to other heat treatable alloys such as the AA2000 and 6000 series aluminum alloys as well as

AA8000 alloys which include lithium, e.g., 8090 and 8091. Thus, typical AA2000 series alloys which may be included are AA2024, 2124, 2324, 2219, 2519, 2014, 2618, 2034, 2090 and 2091, and typical of AA6000 series alloys are 6061 and 6013. Products formed from these alloys have oxygen content of less than 0.1 wt. %. Further, the products, e.g., flat rolled products, are substantially free of the as-cast structure.

As well as providing the alloy product with controlled amounts of alloying elements as described hereinabove, it is preferred that the alloy be prepared according to specific method steps in order to provide the most desirable characteristics of both strength and fracture toughness. Thus, the alloy as described herein can be provided as an ingot or billet for fabrication into a suitable wrought product by casting techniques currently employed in the art for cast products, with continuous casting being preferred. The ingot or billet may be preliminarily worked or shaped to provide suitable stock for subsequent working operations. Prior to the principal working operation, the alloy stock is preferably subjected to homogenization, and preferably at metal temperatures in the range of 850° to 1050° F. for a period of time of at least one hour to dissolve soluble elements and to homogenize the internal structure of the metal. A preferred time period is about 20 hours or more in the homogenization temperature range. Normally, the heat up and homogenization treatment does not have to extend for more than 40 hours; however, longer times are not normally detrimental. A time of 20 to 40 hours at the homogenization temperature has been found quite suitable.

In one aspect of the invention, to produce an unrecrystallized product the ingot may be hot rolled directly to final gauge plate or sheet before being subjected to an isothermal soak and then ramp annealed in accordance with the present invention. Thus, to provide a sheet product or plate in accordance with the invention, particularly thin gauge plate product, the product is subjected to a warm temperature or isothermal soak treatment. Thus, the isothermal soak can be carried out at a temperature as low as 250° F. but normally higher than 275° F. and typically in the range of 300° to 500° F. The soak can be for a time of a few hours, e.g., 3 hours, particularly if the temperature is high and can extend for 24 hours or more. Typically, the soak time extends for 4 to 20 hours. Thereafter, the flat rolled product is subjected to a ramp anneal where the anneal temperature is increased with time of anneal and is carefully controlled until it reaches a higher ending temperature. Preferably, such ending temperatures are in the range of 650° or 700° to 900° F. The starting temperature can be anywhere from about 100° F. in some instances. Typically, the starting temperature will be in the range of 250° to 730° F. with preferred starting temperatures being less than 300° F., but normally in the range of 300° to 500° F. From the starting temperature to the ending temperature, the temperature can be increased at a controlled rate, e.g., at a rate of 2 to 125° F./hr and preferably at a rate of 5° to 80° F./hr. The ramp anneal can include a series of increases in temperature with a holding time at temperature plateau or series of plateaus. Further, it can include even increases in temperature followed by decreases in temperature until the final ending temperature is reached. Also, there may be even holding plateaus at any one or more temperature level. It will be understood that in some cases, as the anneal temperature gets higher, an independent solution heat

treatment may not be necessary but, instead, is included as part of the ramp anneal, as shown in the figure, or the product may be cooled and a separate solution heat treatment, quench and aging performed. The time from the beginning of the ramp anneal to the ending temperature can be as short as two hours or even less to as long as 20 hours or more. Time periods in the range of 3 to 10 hours have been quite suitable with time periods of 4 to 8 hours being found to be useful.

Use of isothermal soak and ramp anneal as disclosed here has been found to be quite beneficial because this process appears to be somewhat insensitive to practices employed to work the ingot.

Unrecrystallized thin gauge plate or sheet product may be produced as in my copending application entitled "Method of Producing Unrecrystallized Thin Gauge Aluminum Products by heat treating and further working", Ser. No. 256,521, filed Oct. 12, 1988, incorporated herein by reference. The thermal and thermo-mechanical steps should be carefully controlled. By unrecrystallized is meant the absence of well-developed grains and the presence of a highly worked structure containing recovered subgrain and retaining as-worked crystallographic texture, i.e., at least 60% of the plate or sheet is free of well-developed grains or retains the as-worked texture. Thus, after homogenization of the ingot and hot rolling, for example, at temperatures in the range of 650° to 850° F., to a slab dimension, the slab is reheated typically to a temperature in the range of 650° to 900° F. and preferably 700° to 800° F. (depending upon composition), for purposes of dissolving or partially dissolving particles that precipitated during the preceding thermal mechanical operation. Reheating can be carried out in a time as short as  $\frac{1}{2}$ , or  $\frac{1}{2}$  hour at temperature, and can extend for 4 hours or more. However, the longer times are not normally necessary. Then, the slab is cooled at a rate sufficient to retain dissolved elements in solution. Preferably, the slab is cold water quenched or rapidly cooled. Thereafter, the slab is subjected to an elevated temperature precipitation heat treatment to precipitate particles in a controlled manner. The precipitation heat treatment can be carried out at a temperature in the range of 200° to 550° F., preferably 350° to 500° F., with typical temperatures being 400° to 500° F. Precipitation heat treatment times at this temperature can range from 5 to 20 hours or longer, and times of from 9 to 15 hours can be quite suitable. After the precipitation heat treatment, the slab is worked or rolled to thin gauge plate or to sheet stock. Thin gauge plate contemplates having a thickness of at least 0.125, typically 0.25 inch or more. The thickness can extend to 0.5 inch or more, for example, 0.75 or 1.0 or even 1.25 inch.

While the slab may be cold rolled at these temperatures, it is preferred that the slab be rolled to final gauge, e.g., thin gauge plate or sheet, using warm rolling practices. Thus, preferably, warm rolling is performed at a temperature of not greater than 550° F. Further, preferably, the temperature at which warm rolling begins is not less than 200° F. Typically, the warm rolling can begin at the precipitation heat treatment temperature. Preferably, the warm rolling temperature should not exceed the precipitation heat treatment temperature. Such temperatures are in the range of about 350° to 500° F. This warm rolling practice contrasts with the prior art which teaches that rolling temperatures should be significantly higher, typically above about 750° F.

In certain alloys, to obtain an unrecrystallized product, it may be desirable to combine these processes. That is, the isothermal soak and ramp anneal may be used in addition to precipitation heat treating intermediate the working steps, and such combination is contemplated within the purview of the invention.

Thereafter, the plate or sheet product is subjected to a solution heat treatment and then cooled, for example, e.g., cold water quenching.

The solution heat treatment is preferably accomplished at a temperature in the range of 800° to 1050° F. and unrecrystallized grain structure is produced. Generally, for sheet gauge, typically times at these temperatures can be relatively short, for example, 5 minutes or even less is adequate. For thin gauge plate, e.g., 0.5 inch, 10 15 the time required may be as much as 2 hours.

To further provide for the desired strength and fracture toughness necessary to the final product and to the operations in forming that product, the product should be rapidly quenched to prevent or minimize uncontrolled precipitation of strengthening phases referred to herein later. Thus, it is preferred in the practice of the present invention that the quenching rate be at least 100° F. per second from solution temperature to a temperature of about 200° F. or lower. A preferred quenching rate is at least 200° F. per second in the temperature range of 900° F. or more to 200° F. or less. After the metal has reached a temperature of about 200° F., it may then be air cooled.

After the alloy product of the present invention has been quenched, it may be subjected to a subsequent aging operation to provide the combination of fracture toughness and strength which are so highly desired in aircraft members. Artificial aging can be accomplished by subjecting the sheet or plate or shaped product to a temperature in the range of 150° to 400° F. for a sufficient period of time to further increase the yield strength. Some compositions of the alloy product are capable of being artificially aged to a yield strength as high as 100 ksi. However, the useful strengths are in the 30 range of 70 to 90 ksi and corresponding fracture toughnesses are in the range of 20 to 50 ksi/in. Preferably, artificial aging is accomplished by subjecting the alloy product to a temperature in the range of 275° to 375° F. for a period of at least 30 minutes. A suitable aging 35 practice contemplates a treatment of about 8 to 24 hours at a temperature of about 325° F. Further, it will be noted that the alloy product in accordance with the present invention may be subjected to any of the typical overaging or underaging treatments well known in the 40 art, including natural aging. However, it is presently believed that natural aging provides the least benefit. Also, while reference has been made herein to single aging steps, multiple aging steps, such as two or three aging steps, are contemplated and stretching or its 45 equivalent working may be used prior to or even after part of such multiple aging steps.

While the invention has been described with respect to sheet and plate, it will be appreciated that its application is not necessarily limited thereto. That is, the process can be applied to extrusions and forgings having alloy compositions referred to herein or responsive to these treatments. In contrast to rolling, for extrusion purposes, it is not difficult to keep the ingot hot, but it is uneconomical to do so because of the slow extruding rates. Consequently, extrusions typically have a recrystallized structure. To provide an unrecrystallized extrusion in accordance with the invention, the process

would include two or more extruding steps. That is, after achieving an ingot temperature of about 700° to 800°, the ingot is extruded to an intermediate cross-sectional area, e.g., to reduce the area 75%. Thereafter, the 5 partially extruded material is subjected to a reheating step, for example, under the same conditions as referred to herein with respect to slab. Also, it is cooled and subjected to an elevated precipitation treatment as referred to for slab, for example. Thereafter, the partial extrusion is further worked or extruded to product form preferably utilizing warm temperatures, for example, under the same conditions referred to for slab being rolled to final gauge. Thereafter, the extrusion may be solution heat treated, quenched and aged to produce an unrecrystallized aluminum alloy extrusion. Because 10 steps in forming forgings are often repeated, the forging operation may be carried out incorporating the procedures set forth for the flat rolled product to produce an unrecrystallized aluminum alloy forged product. It will be appreciated that the rolling, extruding or forging 15 steps may be combined to produce an unrecrystallized product.

An aluminum alloy consisting essentially of, by weight percent, 10 Zn, 1.8 Mg, 1.5 Cu and 0.12 Zr, the balance essentially aluminum and impurities, was cast into an ingot suitable for rolling. The ingot was homogenized and rolled to a 1.5 inch thick slab. The slab was cut into several pieces which were subjected to anneals 20 at temperatures of 750° to 880° F. and then hot rolled to 0.3 inch plate. Thereafter, the 0.3 inch plate was isothermal soaked for 16 hours at 400° F. and then subjected to a ramp anneal starting at 400° F. and ending at 800° F., increase in temperature being made in 4 hours. The 0.3 inch plate was then solution heat treated at 880° F. for 25 1 hour followed by a cold water quench. Examination of the microstructure showed unrecrystallized grain structures which demonstrates the effectiveness of isothermal soaking and ramp annealing in preventing recrystallization.

Having thus described the invention, what is claimed is:

1. A method of producing an unrecrystallized aluminum base, wrought alloy product having improved levels of strength and fracture toughness, the method comprising the steps of:

- (a) providing a body of an aluminum base heat treatable alloy;
- (b) working the body to a wrought product;
- (c) subjecting said product to a soak;
- (d) then subjecting said product to a ramp anneal wherein the annealing temperature is increased during time of anneal; and
- (e) solution heat treating, quenching and aging said product to provide a substantially unrecrystallized wrought product having improved levels of strength and fracture toughness.

2. The method in accordance with claim 1 wherein said working is hot working starting at a temperature in the range of 650° to 850° F.

3. The method in accordance with claim 1 wherein in said ramp anneal the ending temperature is 650° to 900° F.

4. The method in accordance with claim 1 wherein in said ramp anneal the starting temperature is less than 300° F. and the ending temperature is 700° to 900° F.

5. The method in accordance with claim 4 wherein the temperature is increased at 2° to 125° F. per hour.

6. The method in accordance with claim 4 wherein the temperature is increased at 5° to 80° F. per hour.

7. The method in accordance with claim 1 wherein said soak is at a temperature in the range of 300° to 500° F.

8. The method in accordance with claim 1 wherein said soak is an isothermal soak for a period of at least 3 hours.

9. The method in accordance with claim 1 wherein the soak is an isothermal soak for a period of at least 4 hours.

10. The method in accordance with claim 1 wherein the soak is for a period in the range of 4 to 24 hours.

11. The method in accordance with claim 1 wherein the alloy is selected from 2000, 6000 and 7000 type 15 aluminum alloys.

12. The method in accordance with claim 1 wherein the alloy is the Al—Zn—Cu—Mg type.

13. The method in accordance with claim 1 wherein the alloy is selected from 7050, 7150, 7075, 7475, 7049 20 and 7039.

14. The method in accordance with claim 1 wherein the alloy contains 1.0 to 12 wt. % Zn, 0.5 to 4.0 wt. % Mg, max. 3.0 wt. % Cu, max. 1.0 wt. % Mn, max. 0.5 wt. % each of Si, Fe, Cr, Ti, Zr, Sc, and Hf, the balance 25 aluminum and impurities.

15. The method in accordance with claim 1 wherein the alloy contains 7.0 to 9.0 wt. % Zn, 1.5 to 2.5 wt. % Mg, 1.9 to 2.7 wt. % Cu, 0.08 to 0.14 wt. % Zr, max. 0.5 wt. % each of Si, Fe, Cr, Ti, Zr, Sc and Hf, the balance 30 aluminum and impurities.

16. The method in accordance with claim 11 wherein the alloy is selected from 2000 type aluminum alloys.

17. The method in accordance with claim 11 wherein the alloy is selected from 6000 type aluminum alloys. 35

18. The method in accordance with claim 16 wherein the alloy is selected from Aluminum Association alloys: 2024, 2124, 2324, 2219, 2519, 2014 and 2618.

19. The method in accordance with claim 17 wherein the alloy is selected from Aluminum Association alloys 40 6061 and 6013.

20. The method in accordance with claim 1 wherein the wrought product is thin gauge plate having a thickness in the range of 0.25 to 0.75 inch.

21. The method in accordance with claim 1 wherein 45 the wrought product is an extrusion product.

22. The method in accordance with claim 1 wherein the wrought product is a forged product.

23. A method of producing an unrecrystallized Al—Zn—Cu—Mg thin plate or sheet product having 50 improved levels of strength and fracture toughness, the method comprising the steps of:

(a) providing a body of an alloy consisting essentially of 1.0 to 12 wt. % Zn, 0.5 to 4.0 wt. % Mg, max. 3.0 wt. % Cu, max. 1.0 wt. % Mn, max. 0.5 wt. % each 55 of Si, Fe, Cr, Ti, Zr, Sc and Hf, the balance aluminum and impurities;

(b) heating the body to a hot working temperature;

(c) hot rolling the body to said product;

(d) soaking said product in the range of 300° to 500° 60 F. for a period of time in the range of 4 to 24 hours;

(e) then subjecting said product to a ramp anneal starting at a temperature in the range of 300° to 500° F. and ending at a temperature in the range of 700° to 900° F. by increasing the temperature at 2° to 125° F. per hour; and

(f) solution heat treating, quenching and aging said product to provide a substantially unrecrystallized

thin gauge flat rolled product having improved levels of strength and fracture toughness.

24. The method in accordance with claim 23 wherein the plate product has a thickness in the range of 0.25 to 0.75 inch.

25. The method in accordance with claim 23 wherein the alloy is 7050 or 7150.

26. The method in accordance with claim 23 wherein the plate product has a thickness in the range of 0.25 to 10 0.5.

27. The method in accordance with claim 23 wherein the alloy is 7075.

28. The method in accordance with claim 23 wherein the alloy is 7475.

29. A method of producing an unrecrystallized Al—Zn—Cu—Mg thin plate or sheet product having improved levels of strength and fracture toughness, the method comprising the steps of:

(a) providing a body of an alloy consisting essentially of 7.0 to 9.0 wt. % Zn, 1.5 to 2.5 wt. % Mg, 1.9 to 2.7 wt. % Cu, 0.08 to 0.14 wt. % Zr, max. 0.12 wt. % Si; max. 0.15 wt. % Fe, max. 0.10 wt. % Mn, max. 0.06 wt. % Ti, max. 0.04 wt. % Cr, the balance aluminum and incidental elements and impurities;

(b) heating the body to a hot working temperature;

(c) hot rolling the body to said product;

(d) soaking said product in the range of 300° to 500° F. for a period of time in the range of 4 to 24 hours; (e) then subjecting said product to a ramp anneal starting at a temperature in the range of 300° to 500° F. and ending at a temperature in the range of 700° to 900° F. by increasing the temperature at 2° to 125° F. per hour; and

(f) solution heat treating, quenching and aging said product to provide a substantially unrecrystallized thin gauge flat rolled product having improved levels of strength and fracture toughness.

30. A method of producing an unrecrystallized aluminum alloy aircraft structural member having improved levels of strength and fracture toughness, the method comprising the steps of:

(a) providing a body of a heat treatable aluminum base alloy;

(b) working the body to a flat rolled product;

(c) subjecting said product to a soak;

(d) then subjecting said product to a ramp anneal starting at a temperature less than 500° F.;

(e) solution heat treating, quenching and aging said product to provide a substantially unrecrystallized product having improved levels of strength and fracture toughness; and

(f) forming said unrecrystallized product into said aircraft structural member.

31. The method in accordance with claim 30 wherein said working is hot working starting at a temperature in the range of 650° to 850° F.

32. The method in accordance with claim 30 wherein in said ramp anneal the ending temperature is 700° to 900° F.

33. The method in accordance with claim 30 wherein in said ramp anneal the starting temperature is less than 500° F. and the ending temperature is 700° to 900° F.

34. The method in accordance with claim 33 wherein the temperature is increased at 2° to 125° F. per hour.

35. The method in accordance with claim 33 wherein the temperature is increased at 5° to 80° F. per hour.

36. The method in accordance with claim 30 wherein said soak is an isothermal soak at a temperature in the range of 300° to 500° F.

37. The method in accordance with claim 33 wherein said soak is an isothermal soak for a period of at least 3 hours.

38. The method in accordance with claim 30 wherein said working is hot rolling starting at a temperature of not higher than 850° F.

39. The method in accordance with claim 30 wherein said working is hot rolling starting at a temperature of not higher than 800° F.

40. The method in accordance with claim 30 wherein said soak is for at least 4 hours.

41. The method in accordance with claim 30 wherein said soak is for a period in the range of 4 to 24 hours.

42. The method in accordance with claim 30 wherein the alloy is the Al—Zn—Cu—Mg type.

43. The method in accordance with claim 30 wherein the alloy is selected from 7050, 7150, 7075, 7475, 7049 and 7039.

44. The method in accordance with claim 30 wherein the alloy contains 1.0 to 12 wt. % Zn, 0.5 to 4.0 wt. % Mg, max. 3.0 wt. % Cu, max. 1.0 wt. % Mn, max. 0.5 wt. % each of Si, Fe, Cr, Ti, Zr, Sc, and Hf, the balance aluminum and impurities.

45. The method in accordance with claim 30 wherein the alloy contains 7.0 to 9.0 wt. % Zn, 1.5 to 2.5 wt. % Mg, 1.9 to 2.7 wt. % Cu, 0.08 to 0.14 wt. % Zr, max. 0.5 wt. % each of Si, Fe, Cr, Ti, Zr, Sc and Hf, the balance aluminum and impurities.

46. A method of producing an unrecrystallized Al—Zn—Cu—Mg aircraft structural member having improved levels of strength and fracture toughness, the method comprising the steps of:

- (a) providing a body of an alloy consisting essentially of 1.0 to 12 wt. % Zn, 0.5 to 4.0 wt. % Mg, max. 3.0 wt. % Cu, max. 1.0 wt. % Mn, max. 0.5 wt. % each of Si, Fe, Cr, Ti, Zr, Sc, and Hf, the balance aluminum and impurities;
- (b) heating the body to a hot working temperature;
- (c) hot rolling the body to a thin gauge plate product having a thickness of 0.25 to 0.75 inch;
- (d) soaking said plate product in the range of 125° to 500° F. for a period of time in the range of 4 to 24 hours;
- (e) then subjecting said plate product to a ramp anneal starting at a temperature in the range of 250° to 730° F. and ending at a temperature in the range of 650° to 900° F. by increasing the temperature at 2° to 125° F. per hour;
- (f) solution heat treating, quenching and aging said plate to provide a substantially unrecrystallized thin gauge flat rolled product having improved levels of strength and fracture toughness; and
- (g) forming said unrecrystallized plate product into said aircraft structural member.

47. The method in accordance with claim 46 wherein the plate product has a thickness in the range of 0.25 to 0.5 inch.

48. The method in accordance with claim 46 wherein the alloy is 7050 or 7150.

49. The method in accordance with claim 46 wherein the alloy is 7075.

50. The method in accordance with claim 46 wherein the alloy is 7475.

51. An aluminum alloy unrecrystallized aircraft structural member formed from thin gauge unrecrystallized plate provided by soaking the plate followed by a ramp anneal where the temperature is increased during anneal

to about 650° to 850° F., the member consisting essentially of 1.0 to 12 wt. % Zn, 0.5 to 4.0 wt. % Mg, max. 3.0 wt. % Cu, max. 1.0 wt. % Mn, max. 0.5 wt. % each of Si, Fe, Cr, Ti, Zr, Sc, and Hf, the balance aluminum and impurities.

52. An aluminum alloy member in accordance with claim 51 wherein said soak is carried out at a temperature in the range of 125° to 500° F.

53. An aluminum alloy member in accordance with claim 51 wherein said soaking is carried out in the temperature range of 250° to 550° F.

54. An aluminum alloy member in accordance with claim 51 wherein said isothermal soaking is carried out in the temperature range of 300° to 500° F.

55. An aluminum alloy member in accordance with claim 51 wherein the alloy contains 5.7 to 6.9 wt. % Zn, 1.9 to 2.7 wt. % Mg, 1.9 to 2.6 wt. % Cu, 0.05 to 0.15 wt. % Zr, max. 0.12 wt. % Si, max. 0.15 wt. % Fe, max. 0.10 wt. % Mn, max. 0.06 wt. % Ti, max. 0.04 wt. % Cr, the balance aluminum and incidental elements and impurities, the thin gauge plate product having a thickness in the range of 0.25 to 0.5 inch.

56. An aluminum alloy member in accordance with claim 51 wherein the plate is 0.25 to 1.0 inch thick.

57. A method of producing an unrecrystallized Al—Zn—Cu—Mg aircraft structural member having improved levels of strength and fracture toughness, the method comprising the steps of:

- (a) providing a body of an alloy consisting essentially of 7.0 to 9.0 wt. % Zn, 1.5 to 2.5 wt. % Mg, 1.9 to 2.7 wt. % Cu, 0.08 to 0.14 wt. % Zr, max. 0.12 wt. % Si, max. 0.15 wt. % Fe, max. 0.10 wt. % Mn, max. 0.06 wt. % Ti, max. 0.04 wt. % Cr, the balance aluminum and incidental elements and impurities;
- (b) heating the body to a hot working temperature;
- (c) hot rolling the body to a thin gauge plate product having a thickness of 0.25 to 0.75 inch;
- (d) soaking said plate product in the range of 125° to 500° F. for a period of time in the range of 4 to 24 hours;
- (e) then subjecting said plate product to a ramp anneal starting at a temperature in the range of 250° to 730° F. and ending at a temperature in the range of 650° to 900° F. by increasing the temperature at 2° to 125° F. per hour;
- (f) solution heat treating, quenching and aging said plate to provide a substantially unrecrystallized thin gauge flat rolled product having improved levels of strength and fracture toughness; and
- (g) forming said unrecrystallized plate product into said aircraft structural member.

58. An aluminum alloy member in accordance with claim 57 wherein the plate is 0.25 to 0.5 inch thick.

59. The aluminum alloy member in accordance with claim 57 wherein the member is an upper wing skin.

60. An aluminum alloy unrecrystallized aircraft structural member formed from thin gauge unrecrystallized plate provided by soaking the plate followed by a ramp anneal where the temperature is increased during anneal to about 650° to 850° F., the member consisting essentially of aluminum base alloy consisting essentially of 7.0 to 9.0 wt. % Zn, 1.5 to 2.5 wt. % Mg, 1.9 to 2.7 wt. % Cu, 0.08 to 0.14 wt. % Zr, max. 0.12 wt. % Si, max. 0.15 wt. % Fe, max. 0.10 wt. % Mn, max. 0.06 wt. % Ti, max. 0.04 wt. % Cr, the balance aluminum and incidental elements and impurities, the product having a thickness in the range of 0.1 to 0.75 inch.

\* \* \* \* \*